

1,283,354.

E. R. SUTCLIFFE,  
METHOD OF BRIQUETING AND THE PRODUCT,  
APPLICATION FILED MAR. 27, 1915.

Patented Oct. 29, 1918.

Fig.1



Fig. 2



Inventor

E. R. Sutcliffe  
by  
W. E. Evans

Attorney



Witnesses

Robert Owen Hughes  
Stanley Wood

# UNITED STATES PATENT OFFICE.

EDGAR ROUSE SUTCLIFFE, OF LEIGH, ENGLAND, ASSIGNOR TO PURE COAL BRIQUETTES LIMITED, OF CARDIFF, WALES.

## METHOD OF BRIQUETING AND THE PRODUCT.

1,283,354.

Specification of Letters Patent. Patented Oct. 29, 1918.

Application filed March 27, 1915. Serial No. 17,505.

To all whom it may concern:

Be it known that I, EDGAR ROUSE SUTCLIFFE, a subject of the King of Great Britain and Ireland, residing at Leigh, Lancashire, England, have invented an Improved Method of Briqueting and the Product, of which the following is a specification.

This invention relates to an improved method of briqueting carbonaceous substances of the character of coal for the production of blocks or briquets of great hardness and toughness in a manner that is expeditious and effective. It relates to an improvement set forth and claimed in my application filed concurrently herewith, Serial No. 17504.

As disclosed in my said application, the material to be treated is first comminuted to an impalpable powder, *i. e.* one in which the entire body of material, or at least the greater part of such material, will pass a screen of 200-mesh. This product is subjected in segregated masses to a preliminary pressure.

According to the invention I reduce the raw material to be briqueted to a very finely comminuted condition in any suitable apparatus such as a tube mill, and I subject the raw material in this very finely comminuted condition to compression to produce compressed or compacted bodies of any desired shape according to the character and form of the apparatus used for the purpose, and I then break up, crush or disintegrate the compressed bodies so produced into small particles and then subject the product of this preliminary compression and disintegration to a further or final compression, carried out advantageously at a higher degree of pressure than that at which the preliminary compression of the raw material took place.

It is found that a better cohesion and consolidation is secured by such a process of briqueting and a product that is very hard and tough.

The invention is of special utility in the production of large blocks or briquets of coal, which by reason of their heavy weight require to be extremely tough so as effectively to withstand the effects of dumping, in transport of the blocks, but it is also of general application to raw materials capable of being briqueted either with or without a binder or agglutinant of a character suitable to the raw material employed.

The method of the invention is illustrated by way of example and diagrammatically in the accompanying drawings, in which—

Figure 1 represents a diagrammatic section of a hopper and plunger press adapted for the preliminary as well as for the further or final compression according to the method of the invention.

In carrying the invention into effect in the production of large blocks or briquets of coal from coal slack or waste coal, I reduce the material into a very finely comminuted condition or flour. This I effect advantageously in a tube mill, so that the condition of the comminuted substance is such that the greater part will pass through a screen of 200 mesh. I find that the very finely comminuted condition of the raw material is important to insure effective briqueting according to the method of the invention. I then subject the coal in this very finely comminuted condition to a preliminary compression, which may take place in a special press or in the press in which the subsequent or final compression is applied.

It will be understood that the preliminary compression may be carried out under conditions that permit of the lateral expansion of the block under the stresses imposed upon it with a view of securing an effective consolidation of the particles as, for example, when a raw material which binds with difficulty, is treated; but in general, such conditions of pressure in the preliminary compression of the raw material are not essential; while again I may produce blocks or briquets in the preliminary compression, of the same or of a larger size than those produced after breaking up or crushing. I may compress the raw material in the preliminary compression into bodies of any size. I may, for example, produce them in the shape of small spheres or other shaped pieces or bodies, and when so providing them I may entirely dispense with the step of breaking up or crushing the product of the preliminary compression before subjecting it to the further or final compression in molds of larger size.

It is to be observed in this connection that the primary compression must be great enough to effect the expulsion of entrapped and absorbed air from the impalpably powdered fuel and binder, if any, and to develop, to some extent at least, the latent plasticity of this impalpably powdered mass, so that

the primarily formed blocks are quite dense and uniform as a result, though not necessarily so hard as they can be made by primary pressure such as that disclosed in 5 my application filed concurrently herewith and numbered serially 17504.

The product of the preliminary compression being in the form of blocks, cakes, nodules, flakes, or bodies it may then be 10 crushed to small particles of a size, for example, as may pass through a screen of one-quarter-inch mesh, and the material passed through the screen may then be subject to a further or final compression in one or more 15 stages. The breaking up or crushing may be effected in any suitable apparatus, as, for example, by passing the material through a pair of toothed crushing rolls. I prefer in general to effect the pre-pressing so as to 20 produce blocks or nodules instead of flakes.

In Fig. 1 the mold and plungers of a hopper and plunger press suitable alike for carrying out the preliminary compression as well as the further or final compression of 25 the material are diagrammatically represented, in which the very finely divided raw material or the crushed and screened blocks, cakes, nodules, flakes, or bodies being the product of the preliminary compression, are 30 fed into the hopper *e*. I prefer to provide the mold *a* tapering outwardly toward the discharge end, into which the material *d* to be compressed is fed by means of the movable plunger *b*. The blocks are produced by compression of the charges between the movable plungers *b* and *c*. The ends of the respective plungers *b* and *c* are recessed at *b*<sup>1</sup> and *c*<sup>1</sup>, so that thus the rear edge of each block is 35 rounded, while the front protruding edge 40 consequently formed upon the block will be crushed on the final pressure being applied by the plunger *c*. In starting from the position indicated in Fig. 1 the plunger *b* will move forward to feed a further charge into 45 the mouth of the mold *a*, and the plunger *c* will at the same time move forward in the opposite direction so that thus the block at the front end of the mold and which has been produced in the previous compression 50 will be finally compressed, while the first compression is applied to the charge fed into the mold. The plunger *b* will then return for a further charge to be fed into the mold, and upon the plunger *b* again moving forward, the finally compressed block at the 55 front end of the mold will be pushed out of the mold. By so providing the mold tapering outwardly the block on the first compression will have stresses imposed upon it, and upon being forced forward in the mold 60 will be free to expand laterally in the larger part of the mold, so that thus the blocks produced are effectively consolidated and are free from cracks or laminations.

65 I have found in the production of cylind-

rical blocks of 3" in diameter and 2" in depth that a uniform taper in the mold of  $\frac{1}{16}$ th of an inch is sufficient to insure the production of a block under the conditions indicated where the compression is carried out 70 in two stages and the degree of pressure is gradually increased up to a final pressure of 10 tons per square inch and the block moved in the mold in the interval between the stages of compression.

75 It will be understood that the further or final compression may be effected in any other press than that diagrammatically indicated in Fig. 1; for example, the blocks may be conveniently made in a hydraulic press, 80 but in this case also I prefer to provide the molds tapering outwardly toward the discharge end of the mold.

85 It will thus be understood that the further or final compression of the preliminarily compressed and disintegrated raw material may be effected by the methods and means described in the specification of the pending application made by me, Serial No. 17,504, filed March 27, 1915. By the preliminary 90 compression and disintegration of the raw material and the subsequent compression of the resulting product in the manner described, a very hard and tough block of coal 95 may be produced. The hardness and toughness imparted to the block render it possible for large and heavy blocks to be produced which will withstand the effects of dumping in transport without being broken up and shattered. I find that a distinct physical 10 character is imparted to the block produced as the result of the method of the invention, for whereas in the production of blocks or briquets in the hopper and plunger press as represented in Fig. 1, in the utilization of very finely comminuted coal not 10 previously subject to preliminary compression and disintegration, a hard block is produced having a fracture similar to the fracture of freestone, a block produced in 11 the same machine of raw material previously subjected to pressure to form blocks which are then disintegrated will break with a fracture not unlike the fracture of a piece of granite. Such a fracture of the block and 11 its behavior under tests indicates that the method of its consolidation according to the invention imparts to it a physical quality by which it is highly resistant to impact; and thus the method of the invention may 12 be employed for the production of blocks or briquets of large size and weight.

12 The degree of pressure under which the preliminary compression takes place may be relatively low and yet be effective. A pressure of from one to five tons per square inch suffices, but the degree of pressure may be varied according to the raw material employed and its capacity of binding, while the degree of pressure applied for the fur- 13

ther or final compression may be from eight to ten tons per square inch.

It will be understood that one of the objects of the invention is to produce blocks without the necessary use of a binder or agglutinant by the improvement in the method of compressing that is involved in the invention, but in dealing with anthracite or coke, that are consolidated with difficulty or not at all when a binder or agglutinant is not used, I advantageously incorporate the binder or agglutinant with the raw material before the preliminary compression and in a finely comminuated condition.

15 It will, however, be understood that the invention is not confined to the production of the final product in the condition of briquets such as are produced in presses, as the compression of the finely divided and 20 preliminarily pressed raw material may be effected within the retorts or ovens when the product is intended for coking, and in such event the compression of the treated raw material in the condition of small spheres or 25 other shaped pieces may be effected by means similar to that now usually employed for the compression of the charges for coke ovens or retorts. Or again, the compression may be effected by tamping or in large molds or receptacles destined to be passed into the ovens or retorts, or the treated raw material may be coked without being subjected to any further compression.

The method of the invention is of general 35 application to raw materials capable of being briqueted, such as minerals, ores, ores or minerals and fuel, cement raw material, or cement raw material and fuel, or raw material for the manufacture of bricks, and 40 when treating such mixtures I may reduce the several raw materials to a finely comminuted condition separately or together, and otherwise treat them in the manner hereinbefore described with or without a binder 45 as may be necessary according to the character of the raw material.

The hard and tough blocks produced according to the process of the invention may be coked for the production of a coke fuel.

50 I claim:

1. A method of briquetting carbonaceous substances of the character of coal, consisting in reducing the substance to the uniform condition of extreme fineness, subjecting the 55 said substance in the said condition to a preliminary compression, breaking up the compressed product, and subjecting the resulting product to further compression to produce a block or briquet, substantially as described.

2. A method of briquetting carbonaceous substances of the character of coal, consisting in reducing the substance to be briquetted and a binder to the substantially uniform condition of extreme fineness, subjecting the 65 mixture of the said substance and the said binder to a preliminary compression, breaking up the compressed product, and subjecting the resulting product to further compression to produce a block or briquet, substantially as described.

3. A method of briquetting carbonaceous substances of the character of coal, consisting in reducing the substance to be briquetted to the substantially uniform condition of extreme fineness, subjecting the said substance in said condition to a preliminary compression, breaking up the compressed product, subjecting the resulting product to further compression, and permitting the expansion 75 of the block or briquet transversely to the line of application of the pressure under the stresses imposed in the said further compression, substantially as described.

4. A method of briquetting carbonaceous 85 substances of the character of coal, consisting in reducing the substance to be briquetted to the uniform condition of extreme fineness, subjecting the said substance in the said condition to a preliminary compression, 90 breaking up the compressed product, subjecting the resulting product to a further compression in a plurality of stages, and permitting the expansion of the block or briquet in the interval between the successive stages of compression transversely to 95 the line of application of the pressure employed, substantially as described.

5. As a new article of manufacture, a 100 hard and tough briquet composed of a carbonaceous substance compressed in a dry state to coherence from a uniform condition of extreme fineness, and again subjected, when in the shape of lumps or fragments, to 105 compression in mass, substantially as described.

6. A method of briquetting carbonaceous material which consists in reducing said material to a uniform condition of extreme fineness, compressing said material, when in 110 such condition, dry to compactness and coherence, and recompressing and compacting such compressed and compacted material, when it is in the condition of lumps or fragments, to produce dense, compact blocks or 115 briquets, substantially as described.

EDGAR ROUSE SUTCLIFFE.

Witnesses:

WILLIAM EDWARD EVANS,  
ROBERT OWEN HUGHES.